

Jan. 3, 1928.

1,654,624

S. D. WELLS

PROCESS OF SEPARATING VEGETABLE FIBROUS MATERIAL

Filed Aug. 10, 1925



By Sidney D. Wells  
William L. Symmons  
his Attorney

Inventor

## UNITED STATES PATENT OFFICE.

SIDNEY D. WELLS, OF QUINCY, ILLINOIS.

## PROCESS OF SEPARATING VEGETABLE FIBROUS MATERIAL.

Application filed August 10, 1925. Serial No. 49,461.

This invention relates to the production of fiber suitable for manufacture of paper and pertains particularly to the treatment of wood and other vegetable fibrous material by the steps of the particular process and within a certain apparatus, both of which comprise a part of the present invention.

The process provides for the treatment of softened woody material and which has been converted into a ligno-cellulosic intermediate product by pounding and rubbing such previously prepared material into pulp in a particular way without breaking the fibers and without the reduction to fragments of more than an insignificant proportion of the fibers and cells.

The apparatus provides a rotatable drum structure within which the pulp is tumbled, pounded and beaten by intermingling contact with a plurality of rods which extend in parallel relation lengthwise of the axis of the drum and are free to roll and tumble therein under the influence of the rotary movement of the drum. With this improved pulping apparatus the length of the fiber is maintained and the fibers are not disintegrated into the sawdust-like particles commonly produced and observed in processes in which the grinding apparatus includes a rotary abrading element or cutting element.

Especially does this invention relate to the mechanical phases of fiber producing processes and to the resulting fibrous material suitable for paper manufacture and for other purposes, obtained from wood as for example after the original material has been prepared chemically by boiling the same under pressure in the presence of aqueous solutions of caustic soda and sodium sulphide, caustic soda and sulphur, or sodium sulphite and sodium carbonate of suitable concentration to soften the woody material and to form the lingo-cellulosic intermediate product above mentioned.

At the present state of the pulp makers' art the processes used may be divided into two groups, the mechanical and the chemical. The mechanical process consists essentially of pressing blocks of wood against a revolving grindstone in the presence of water and the wood is reduced to pulp by grinding and the frictional heat developed. In this process the action is so severe that compara-

tively few of the fibers survive in their entity and a large portion of the pulp consists of fragments of single fibers or of bundles of fibers. In the chemical processes the wood is cut to chips and digested under pressure in aqueous solutions of the bisulphites of the alkaline earths and sulphurous acid or caustic soda or caustic soda and sodium sulphide or sodium sulphite. The digestion is carried to such a point that over fifty per cent of the wood substance is dissolved and a product testing over 90% cellulose is left. In these processes the ultimate fibers are intact, but the bond between them has been removed so that they separate with the slightest mechanical agitation. By ultimate fiber is meant the elongated cells which are attached longitudinally and cemented together radially by incrusting matter consisting largely of lignin and hemicelluloses. Their entity is readily discernible under the microscope and their length is approximately 100 times or more their diameter.

In the present improvement the wood is also cut to chips and the chips subjected to aqueous solutions of suitable chemicals at elevated temperatures after first being subjected to an impregnation treatment under pressure. The digestion however is only carried to the point that the middle lamella or cementing material between the fibers is softened, but not completely dissolved. The softened chips are then capable of reduction to their ultimate fibers and cells by suitable pounding or rubbing or a combination of both in accordance with the present invention. A pulp is obtained that has the general appearance of pulp obtained by the chemical processes mentioned, but instead of a yield of from 40 to 50 per cent being obtained, a yield of from 60 to 85 per cent is realized, depending on the species of wood and the severity of the treatment. While these pulps are similar in appearance to what are generally known as chemical pulps they have distinct chemical characteristics, as will be shown in the following table of analysis. In this table the terms used may be explained as follows:

*Solubility in 1% sodium hydroxide.*—This test is the amount of material dissolved on treatment of the pulp one hour in a 1% solution of sodium hydroxide at 100° C.

*Cellulose.*—The cellulose is determined by subjecting the material to alternate treatments with chlorine gas in the presence of water and washing with sodium sulphite solutions under the conditions suggested by Cross and Bevan and described by A. W. Schorger Jour. Ind. and Eng. Chem. 9, (1917) 556. In accordance with this, the following procedure is used. Two grams of air dry pulp in an alundum crucible are extracted three to four hours with a mixture of 67 per cent of benzol and 33 per cent alcohol. After evaporation of the solvent the shavings are thoroughly washed with hot water using the suction pump. The moist pulp is then transferred with a pointed glass rod to a 250 cc. beaker, evenly distributed over the bottom, and subjected to a stream (about forty bubbles per minute for each sample) of water washed chlorine gas for half an hour. The end of the tube delivering the chlorine gas should be about one-half inch above the pulp. At intervals of six to seven minutes the contents of the beaker are stirred to insure uniformity of chlorination. After the chlorine treatment the pulp is treated with a solution of  $\text{SO}_2$  until the chlorine odor disappears, transferred to the alundum crucible, and washed with hot water. The pulp is again returned with the glass rod to the beaker, and 100 cc. of a two per cent sodium sulphite solution are added and the beaker, covered with a watch glass, placed in a boiling water bath for 30 minutes. The fibers are then transferred to the crucible and washed with water. The above procedure is seldom sufficient to remove all the lignin, so that the treatment with chlorine and subsequent treatment as outlined above is repeated until the fibers are practically a uniform white. The second and following treatments with chlorine should not be longer than 15 to 30 minutes. After all the lignin has been removed the fibers are given a final bleaching by adding 20 cc. of a 0.1 per cent solution of potassium permanganate, allowed to stand 10 minutes and rendered colorless with  $\text{SO}_2$  solution. The fibers are then thoroughly washed with hot water, dilute acetic acid, then with hot water, then with alcohol and finally with ether, and dried for two hours at  $105^\circ \text{ C}$ . in the air oven. After cooling by a desiccator over  $\text{H}_2\text{SO}_4$ , the crucible is weighed in a weighing bottle.

*Lignin.*—This result consists of the residue left after treatment with sulphuric acid under conditions prescribed by Ost and Wilkening and reported by Cross and Bevan in "Researches on Cellulose", III, 39, (1906-10). In adapting that method to the present problems the following steps are followed. Two to four grams of air dry pulp are weighed in an alundum thimble, extracted with ether in a oxlet apparatus for 3 to 4 hours, and dried at  $105^\circ \text{ C}$ . The pulp is then

removed from the alundum extraction thimbles, placed in 250 cc. beakers, divided into fine particles and treated with 40 cc. of 72.0 per cent sulphuric acid. The hydrolysis is allowed to proceed for 16 hours at room temperature, with frequent stirring at the beginning of the operation. The resulting solution is transferred to a two liter Erlenmeyer flask diluted to 1570 cc. with distilled water, which makes the concentration of  $\text{H}_2\text{SO}_4$  exactly 3 per cent, and boiled under a reflex condenser for two hours. This causes a coagulation of the suspended particles of lignin, which is then filtered on an alundum crucible, washed thoroughly with hot water, dried and weighed as lignin.

| Material analyzed                                                 | Soluble in 1% sodium hydroxide |          | Cellulose | Lignin | 85 |
|-------------------------------------------------------------------|--------------------------------|----------|-----------|--------|----|
|                                                                   | Per cent                       | Per cent |           |        |    |
| Wood:                                                             |                                |          |           |        |    |
| Aspen                                                             | 20                             | 62       | 23        |        |    |
| Spruce                                                            | 15                             | 58       | 28        |        |    |
| Loblolly pine                                                     | 13                             | 60       | 30        |        |    |
| Jack pine                                                         | 16                             | 60       | 33        | 90     |    |
| Mechanical pulp: Spruce                                           | 10                             | 60       | 30        |        |    |
| Very raw sulphite pulp: Spruce                                    | 13                             | 77       | 17        |        |    |
| Standard sulphite pulp: Spruce                                    | 12                             | 93       | 4         |        |    |
| Soda pulp:                                                        |                                |          |           |        |    |
| Spruce                                                            | 5                              | 94       | 4         |        |    |
| Jack pine                                                         | 4                              | 94       | 6         |        |    |
| Loblolly pine                                                     | 3                              | 92       | 5         |        |    |
| Aspen                                                             | 2                              | 97       | 2         | 95     |    |
| Sulphate pulp:                                                    |                                |          |           |        |    |
| Spruce                                                            | 6                              | 95       | 3         |        |    |
| Jack pine                                                         | 3                              | 94       | 6         |        |    |
| Loblolly pine                                                     | 2                              | 94       | 6         |        |    |
| Longleaf pine                                                     | 3                              | 94       | 5         |        |    |
| Ligno-cellulosic material, strongly alkaline reagents:            |                                |          |           |        |    |
| Aspen (soda liquor)                                               | 2-9                            | 91-70    | 8-23      | 100    |    |
| Loblolly pine (soda liquor)                                       | 4-7                            | 80-64    | 20-31     |        |    |
| Jack pine (soda liquor)                                           | 3-6                            | 80-63    | 23-32     |        |    |
| Jack pine (sulphate liquor)                                       | 4-7                            | 80-66    | 20-30     |        |    |
| Ligno-cellulosic material, neutral or slightly alkaline reagents: |                                |          |           |        |    |
| Aspen                                                             | 6                              | 74       | 19        |        |    |
| Tupelo gum                                                        | 5                              | 70       | 14        |        |    |
| Chestnut                                                          | 8                              | 77       | 18        | 105    |    |
| Jack pine                                                         | 5                              | 75       | 22        |        |    |
| Loblolly pine                                                     | 4                              | 68       | 28        |        |    |
| Tamarack                                                          | 5                              | 71       | 23        |        |    |

The ligno-cellulosic material may be differentiated from mechanical pulps in that they contain less than 10% of substances soluble in 1% caustic soda solution and 80% or more of the fibers retain 50% or more of their ultimate fiber length. It may be differentiated from the sulphite pulps of commerce in that when obtained from deciduous wood, they are not more than 9% soluble in 1% caustic soda solution, contain from 70% to 91% cellulose, and from 8% to 23% of lignin. It may be differentiated from the soda or sulphate pulps of commerce in that they contain less than 91% cellulose and more than 8% of lignin. When derived from coniferous species they contain from 63% to 80% of cellulose and from 20% to 32% of lignin and is not more than 7% soluble in sodium hydroxide.

The chemical treatment thus far described is not a part of the present invention but is described and claimed in the copending ap-

lication filed jointly by the applicant herein with John D. Rue and Francis G. Rawling, Serial No. 127,178, filed Aug. 4, 1926, and which was predicated on and copied in 5 part from this present application.

An important element of novelty in the present process is the use of mechanical disintegrating types of apparatus in the process which have never before been used on this 10 sort of material for the purpose. The beaters, refining engines or attrition mills fitted with rigid bars or blades which have been used in the paper making art have been found to produce a very unsatisfactory material when applied to softened woody material. 15 Vascular bundles and fragments of the medullary rays are produced which resist reduction longitudinally and appear in the sheet of paper formed from the resultant product as granular sawdust like specks or slivers which render it practically useless for the purpose intended. If the grinding is carried on to the point where these particles have been satisfactorily reduced in size the fibers are also reduced in 20 length until they have lost their power of imparting the desired strength to the paper. On the other hand when properly reduced by pounding or rubbing these fragments do not appear in the finished product and a sheet of 25 uniform texture may be obtained. Not only may this pounding or rubbing action be applied to softened woody material, but it may be applied with excellent results to the beating 30 of the standard chemical pulps or rag or rope or jute pulps of commerce. The rod mill has been found most satisfactory for 35 this purpose.

The process is carried out with the use of 40 particular apparatus which is used for providing the pounding or rubbing action and which apparatus is identified, as above mentioned, as a rod mill. The structure of this apparatus will be briefly described by reference to the accompanying sheet of drawings 45 in which:

Figure 1 represents a top plan view showing an elongated cylindrical drum which is mounted at either end in suitable supporting bearings, and which is shown as having 50 adjacent one end a large gear encircling it, the teeth of which are enmeshed with a smaller gear driven from any suitable source of power;

Figure 2 is a vertical longitudinal section along the line 2—2 of Figure 1 illustrating the intake and outlet openings of the drum and showing the position within the drum of a plurality of long rods which lie free to 55 roll and tumble during the rotary movement of the drum; and

Figure 3 is a sectional view taken on the line 3—3 of Figure 1 vertically and transversely through the drum showing the position of 60 the rods during the revolution of the drum.

Referring in detail to the several figures in the drawing, 1 indicates the cylindrical-like shell of a rotary drum which is mounted with its longitudinal axis extending substantially horizontally and supported in bearings 70 2 at either end on upright supports 3. 4 indicates a large annular gear secured to the flange at one end of the drum. In mesh with the teeth of the gear 4 is a smaller gear 4<sup>a</sup> which is driven by any suitable source of 75 power through a shaft 4<sup>b</sup> and pulley wheel 4<sup>c</sup>.

The intake end 5 receives chips which may or may not have been previously softened, but preferably this material is softened in accordance with the several steps outlined in 80 the description hereinafter provided. During the revolution of the drum 1 the material works its way gradually toward the outlet end and discharges through the opening 6, the rate of discharge being proportional 85 with the rate of intake. A plurality of rods 7 in number sufficient to half fill the drum lie along the bottom and on top of each other. These rods are preferably from one to two 90 inches in diameter and have a length about two inches shorter than the inside length of the drum. The inner lining of the drum may have a contour variable according to the type of fiber to be treated. A so-called "wave" type shell liner has operated to advantage, and in this particular form there are occasional rounded humps which extend lengthwise of the shell or drum wall and aid in lifting the rods and fibrous material 95 from the bottom during the revolution of the structure. The smooth surface of the wave type lining is useful in maintaining uninjured the full length of the fibers, contrasted to which angular linings tend to cut and 100 destroy the fibers.

During the operation of the apparatus, the rods and fibrous material are lifted upward with the movement of the casing and the entire mass of fibrous material intermixed with the rods rolls from top to bottom of the 110 pile toward the opposite side of the drum. This rolling and tumbling movement of the rods serves to rub, pound and beat the previously softened vegetable fiber material into a relatively open condition, thus providing 115 a satisfactory pulp. It is obvious that there is little if any cutting action detrimental to the felting property of the fibers, and it is also obvious that as long as there are any unreduced bundles or lumps in the mass, 120 they will receive substantially the entire action of the rods and correspondingly the portions that are sufficiently reduced will be protected by the lumps and will escape further reduction. It is therefore obvious that the rod mill is selective in its action and consequently attains its results with the least expenditure of energy on material already in 125 proper condition. It is thus also different from positively operated types of equipment 130

now in use for beating or grinding paper pulp.

The action of the rods in the rod mill on the particles of vegetable material may be compared to the treatment which the particles would receive on an inclined surface while pounding elements roll from top to bottom across the inclined surface, rolling, crushing and pounding the particles as the rods tumble from top to bottom. The pile of rods maintains more or less a uniform inclined surface, but as regards the relation of one rod to another, the mass or pile of rods is in constant transition, the rod elements moving from the bottom of the pile toward the crest of the pile, being carried upward by the rotation of the casing, successive rods, after reaching the crest of the pile, being carried so high that the uppermost rod is carried so far that it is no longer retained by the rods next beneath, but falls downward across the inclined surface of the more slowly moving rods until it reaches the side of the pile and comes to rest adjacent to the casing on the side thereof opposite to that from whence it started. In the constant transition of individual elements of the pile of rods from bottom to top, and thence more rapidly across the inclined face of the pile of rods, it will be obvious that the respective rods making up the inclined face also are moving downward, although the largest number of the rods thus forming the inclined surface move more slowly than the ones which are carried to the extreme crest or top of the pile, and which tumble across the surface to the opposite side. It will also be obvious that the plurality of rods composing the inclined surface provide a corrugated effect. Accordingly, particles of vegetable material appearing on the inclined surface of the pile of rods are subjected to the impact of the rapidly moving rods as they are released from the top side and roll across the corrugated surface toward the lower side, striking and rolling across the outer side of each of the individual elements thus forming the corrugated surface. It will also be obvious that not only will the particles of vegetable material be given a peculiar treatment in between the rods and within the mass of the rods by reason of the constant transition movement of the shifting body of rods, but also that an unusual impact treatment is given to all particles of the vegetable material which lie on the upper surface, and such upper particles receive an impact treatment due to the direct contact of a freely moving, falling, tumbling body.

The following procedure may be used in treating fresh wood fibrous material to produce the ligno-cellulosic material described. The wood is first converted to chips in the manner used in chemical pulp mills and charged into a digester. They are then impregnated by steaming and then forcing the softening solution into them by filling the digester therewith and producing hydrostatic pressure by means of a pump, steam, air, or any other method known to the art. After impregnation for half an hour or more at 100 pounds pressure the softening solution will be found to have practically penetrated the chips and the excess over that required for softening is removed. Using 10 parts of sodium sulphite and 4 parts of sodium bicarbonate per 100 parts dry weight of gum chips gave excellent results. The substitution of sodium carbonate for bicarbonate was also satisfactory. The substitution of 2 parts caustic soda for the bicarbonate gave satisfactory results with loblolly pine. For pulps from the pines where greater strength is desired 8 parts of caustic soda and one part of sulphur was satisfactory. 8% calcium bisulphite and 2% sulphurous acid gave good results with tamarack. It can thus be seen that a wide range of chemicals may be used. This impregnation feature is important because it makes possible the softening of the wood uniformly through its thickness. By the term "uniform" is meant the even softening to substantially the same degree from the exterior to the center of each piece of wood. Thus, the chips after treatment are practically as soft at their centers as they are on the outside. Without previous impregnation and with the use of the direct cook only, the woody material is likely to become damaged by over cooking on the exterior portions before the interior is adequately softened. Thus, with ordinary cooking methods, the undigested chips will be almost completely cooked on the outside, and in extreme cases, the center will be bright wood, not even discolored by the cooking liquor. Accordingly, in view of the fact that the particular subsequent mechanical separation of this invention requires uniform softening, it becomes extremely important that the softening step to be conducted in accordance with the procedure herein prescribed.

After the excess of liquor has been withdrawn the contents of the digester are heated until a temperature of over 120° C. has been attained and the contents held thereat until the desired softening has taken place. In the first three instances two hours at 160° C. was sufficient. Four hours at 160° C. was sufficient in the fourth, and six hours coming up to a temperature of 120° C. was sufficient in the last. The contents are then removed from the digester and reduced to ultimate fibers by passing through the rod mill of the present invention. The pulps produced are then washed and prepared in suitable form by the customary steps used in the art. In the use of rubbing and pounding devices screens are desirable to allow the

ultimate fibers or cells to pass on and return the material insufficiently disintegrated for additional rubbing and pounding thereby forming a closed system.

Not only is the rod mill adapted to pulping wood but it is also adapted for use in pulping cooked or softened cereal straws, and also bamboo, cornstalks, bagasse from sugar cane, sorghum, flax straw, hemp, alfagrass, palmetto, palm, saw grass, cane, and in fact almost any of the fibrous plant materials may be so treated. Not only may softened fibrous plant material be treated in the rod mill, but the softening can be accomplished while the material is being rubbed or pounded by admitting hot water or blowing steam into the mill to maintain an elevated temperature and at the same time admit sodium carbonate, milk of lime or any of the known softening agents or mixtures thereof with the raw fiber.

Not only is the rod mill treatment suitable for rubbing apart the fibers in softened fibrous material or for both softening and rubbing where the material is to be used for paper manufacture in the unbleached and unpurified condition, but it may be used where the product therefrom is to be further purified by washing, treatment with chlorine gas or chlorine water, boiled with sodium sulphite, sodium carbonate, sodium hydroxide or some similar compound capable of dissolving the products of chlorination. The fibrous product may then be subjected to a repetition of the same treatment and then bleached by customary methods or when not necessary the repetition of the chlorination treatment may be omitted. The purification processes outlined above are not claimed except in so far as the rod mill is used to prepare the material into proper condition without which these processes are unsatisfactory. The use of the rod mill in preparing lime cooked straw for paper products or for further purification by means of chlorination methods is particularly important.

Should a mixture of coniferous and deciduous material be treated in accordance with the process of this invention, the resultant ligno-cellulosic pulped material would have varying proportions of lignin and cellulose in its content, ranging from 8 per cent to 32 per cent of lignin and from 63 per cent to 91 per cent of cellulose, depending on the ratio of coniferous and deciduous material present.

I claim:

1. In the production of fibers from vegetable material for use in making paper, the method of treating material which has been uniformly softened but not pulped, which method consists in separating the fibers of said softened material by pounding the same between parallel pounding surfaces of a plu-

rality of elongated pounding elements which extend in substantial constant parallel relation and which freely fall in intermingled contact with the material and impact upon particles of the material.

2. In the production of fibers from vegetable material for use in making paper, the method of treating material which has been cooked with chemicals until the middle lamella is softened and which cook has been terminated before the middle lamella is completely dissolved, which method consists in separating the fibers of said softened material by pounding the same between parallel pounding surfaces of a pile of rods which substantially constantly extend parallel to each other and are tumbled with the material and which fall with the material and impact upon particles of the material, whereby the length of the fibers is maintained.

3. In the production of fibers from vegetable material for use in making paper, the method of treating material which has been softened but not pulped, which method consists in subjecting the vegetable fibrous material to a mechanical treatment in which the chemically treated fibrous material which has been softened is commingled with a pile of loose pounding elements comprising parallel rods extending substantially constantly and substantially horizontally and the commingled mass is tumbled in a rotary drum mounted to turn on an axis parallel to the length of the rods whereby the previously softened fibers are pounded between falling parallel surfaces and the fibers are separated from each other.

4. In the production of fibers from vegetable material for use in making paper, the method of treating vegetable particles to loosen the fibers thereof which method consists in pounding particles of the fibrous material between parallel pounding surfaces of a plurality of elongated pounding elements which extend in substantially constantly parallel relation and which freely fall in intermingled contact with the fibrous material and within a restricted zone and impact on particles of the material.

5. In the production of fibers from vegetable material the method of treating vegetable particles to loosen the fibers thereof which method consists in subjecting the fibrous material in a drum mill having freely tumbling disintegrating rods therein to a tumbling action in intermingled contact with said rods while the drum mill is rotated on an axis parallel to the axis of the rods whereby the mass of rods and fibrous material is lifted and permitted to tumble downwardly from that side of the interior of the drum on which it is lifted.

6. In the production of paper pulp from vegetable material, the method of pounding

- 5 apart fibre bundles which method comprises subjecting particles of the vegetable material to a crushing treatment on the inclined upper surface of a pile of elongated pounding elements arranged with their longest axes substantially parallel to each other and horizontal and between said surface and a number of rapidly moving like elements falling from the upper side of the pile to-  
 10 ward the lower side, and constantly moving elements from the lower side of the pile to the upper side and constantly releasing elements at the upper side to roll downward across the particles of vegetable material  
 15 on said inclined surface.

7. In the production of paper pulp from vegetable material, the method of pounding apart fibre bundles which method comprises subjecting particles of the vegetable material to a crushing treatment on the inclined upper surface of a pile of elongated pounding elements arranged with their longest axes substantially parallel to each other and horizontal and between said surface and a  
 20 number of rapidly moving like elements falling from the upper side of the pile toward the lower side, and constantly moving elements from the lower side of the pile to the upper side and constantly releasing elements  
 25 at the upper side to roll downward across the particles of vegetable material on said inclined surface, the plurality of elements of said inclined surface constituting a corrugated surface on which the vegetable par-  
 30 ticles are pounded.

8. In the production of paper pulp from vegetable material, the method of pounding apart fibre bundles which method comprises subjecting particles of the vegetable material to a crushing treatment on the inclined upper surface of a pile of elongated pounding elements arranged with their longest axes substantially parallel to each other and horizontal and between said surface and a  
 40 number of rapidly moving like elements falling from the upper side of the pile to-  
 45 ward the lower side, said pile being in constant transition during conduct of the method and in which transition elements from the lower part of the pile are moved on the side opposite to said inclined surface upwardly to the crest of the pile, thence, to tumble downwardly to impact on the vegetable particles, remaining constantly parallel throughout the movement.

9. In the production of paper pulp from vegetable material, the method of pounding apart fibre bundles which method comprises subjecting particles of the vegetable material to a crushing treatment on the inclined upper surface of a pile of elongated pounding elements arranged with their longest axes substantially parallel to each other and horizontal and between said surface and a  
 60 number of rapidly moving like elements fall-  
 65 ing from the upper side of the pile toward the lower side, and constantly moving elements from the lower side of the pile to the upper side and constantly releasing elements at the upper side to roll downward across the particles of fibrous material on said inclined surface.

10. In the production of products from fibrous materials, the method of beating which consists of pounding the fibers be-  
 70 tween parallel pounding surfaces of a plu-  
 75 rality of elongated pounding elements which extend in substantially constantly parallel relation and which freely fall in intermingled contact with the fibrous material and within a restricted zone and impact on par-  
 80 ticles of the material.

11. In the production of products from fibrous materials, the method of beating which consists in subjecting the fibers in a drum mill having freely tumbling disinte-  
 90 grating rods therein to a tumbling action in intermingled contact with said rods while the drum mill is rotated on an axis parallel to the axis of the rods whereby the mass of rods and fibrous material is lifted and per-  
 95 mitted to tumble downwardly from that side of the interior of the drum on which it is 100 lifted.

12. In the production of products from fibrous materials, the method of beating which consists of subjecting the fibers to a crushing treatment on the inclined upper 105 surface of a pile of elongated pounding elements arranged with their longest axes sub-  
 110 stantially parallel to each other and hori-  
 115 zontal and between said surface and a num-  
 120 ber of rapidly moving like elements falling from the upper side of the pile toward the lower side, and constantly moving elements from the lower side of the pile to the upper side and constantly releasing elements at the upper side to roll downward across the 125 particles of fibrous material on said inclined surface.

13. In the production of products from fibrous materials, the method of beating which consists of subjecting the fibers to a 120 crushing treatment on the inclined upper surface of a pile of elongated pounding elements arranged with their longest axes sub-  
 125 stantially parallel to each other and hori-  
 130 zontal and between said surface and a num-  
 135 ber of rapidly moving like elements falling from the upper side of the pile toward the lower side, and constantly moving elements from the lower side of the pile to the upper side and constantly releasing elements at the 140

upper side to roll downward across the particles of fibrous material on said inclined surface, the plurality of elements of said inclined surface constituting a corrugated 5 surface on which the fibrous particles are pounded.

14. In the production of products from fibrous materials, the method of beating which consists of subjecting the fibers to a 10 crushing treatment on the inclined upper surface of a pile of elongated pounding elements arranged with their longest axes substantially parallel to each other and horizontal and between said surface and a num-

ber of rapidly moving like elements falling 15 from the upper side of the pile toward the lower side, said pile being in constant transition during conduct of the method and in which transition elements from the lower part of the pile are moved on the side opposite to said inclined surface upwardly to the crest of the pile, thence, to tumble downwardly to impact on the fibrous particles, remaining constantly parallel throughout the movement.

In testimony whereof I affix my signature.

SIDNEY D. WELLS.